

## UNITED STATES PATENT OFFICE

2,516,083

TRANSPARENTIZING REGENERATED  
CELLULOSE SILK

Ernst Weiss, Wattwil, Switzerland, assignor to  
Heberlein Patent Corporation, New York, N. Y.,  
a corporation of New York

No Drawing. Application December 22, 1945, Se-  
rial No. 637,119. In Switzerland December 27,  
1944

4 Claims. (Cl. 8—118)

1

This invention relates to a process for transparentizing fibers and fabrics of regenerated cellulose.

Transparentizing of cotton fabrics by means of sulfuric acid is known and has been used extensively commercially. Transparentizing of artificial silk, namely, regenerated cellulose silk fabrics with swelling agents is known, but due to the ease with which sulfuric acid and other swelling agents proposed attack the regenerated cellulose, it has been difficult to control such processes to produce a transparentization, either in all-over or pattern effect, having the same uniform appearance and high quality obtainable by the process as applied to cotton. Attempts to secure greater uniformity and to lessen the vigorous action of the sulfuric acid have been proposed by combining with the acid substances, such as monovalent or multivalent alcohols, heterocyclic bases, formaldehyde, ammonia salts, urea and their derivative amino compounds. But these processes have not given the desired results to produce a satisfactory commercial transparentized viscose or other regenerated cellulose in transparent form.

The principal object of the invention accordingly is to provide a process for the treatment of regenerated cellulose silk, such as viscose, which may be easily controlled to produce a transparentized regenerated cellulose of high quality and appearance.

I have found, unexpectedly in accordance with my invention, that the above difficulties may be overcome by giving such fibers or fabrics a transparentizing treatment, followed by a treatment which has the result of making the fabric appear more uniform and to give it a high quality both as to strength and appearance. This may be most satisfactorily done by the use of caustic potash used, in accordance with my invention, at a regulated range of temperature, time and concentration. And I have found also that the caustic solution should be removed as rapidly as possible, for example, by means of hot rinsing. The concentrations of potassium hydroxide which may be employed are preferably quite high, namely, of the order of 30° Baumé. Room temperature is preferably used. Instead of caustic potash, caustic soda of a much lower concentration may be used, namely, 6 to less than 12° Baumé. Room temperature is also used. The treatment is followed by washing with boiling water to eliminate the caustic soda. The caustic alkali solutions are used under conditions of time, temperature and concentration such that the solutions are incapable of producing a parch-

2

mentizing effect on the original untreated regenerated cellulose. The use of caustic potash and caustic soda in the concentrations mentioned is in accordance with the known solubilities of regenerated cellulose, such as viscose in aqueous solutions of these alkalies. Potassium hydroxide has a far lower dissolving power for regenerated cellulose, dissolving (when about 4.5 N KOH is used) only about 6% thereof as compared with 90% for sodium hydroxide (using about 2.5 N NaOH) at 0° C. In the case of both caustic potash and caustic soda solution, the dissolving power decreases as the temperature rises. I take advantage of these facts, in accordance with my invention, to avoid the use of either caustic potash or caustic soda in concentrations and at temperatures which will cause any substantial dissolving of regenerated cellulose material. In other words, after applying the sulfuric acid or other transparentizing treatment which in itself constitutes a partial solution of the cellulose I avoid in the after-treatment with the caustic a further dissolving action. Accordingly, I employ these caustic alkalies under conditions such that this second dissolving action is substantially avoided.

As a result I obtain transparentized regenerated cellulose which has a uniform and otherwise pleasant appearance and is of high quality, i. e., it has good wearing qualities and has a relatively soft feel, due probably to the fact that the second caustic treatment is not a dissolving treatment since it appears that each dissolving treatment tends to stiffen and otherwise impair the material somewhat. By my process only one such dissolving treatment is effected, and accordingly only a limited stiffening occurs.

My process is suitable for the production of both all-over effects and for local transparent effects with the use of water-soluble or water-insoluble resists and with dyes or pigments as may be desired.

The process is applicable to the treatment of all fine fabrics made from regenerated cellulose, such as spun rayon muslin or viscose muslin, or corresponding voiles.

As transparentizing or parchmentizing agents there may be used the well-known cellulose swelling agents such as sulfuric acid (with or without additions) of over 42° Baumé, phosphoric acid of over 50° Baumé, hydrochloric acid of over 20° Baumé, zinc chloride solutions of over 50° Baumé, calcium thiocyanate solutions of over 25° Baumé, in which connection the requisite concentrations are in addition dependent also upon the reaction

temperature. By such transparentizing treatment, a parchmentized regenerated cellulose textile material results which lacks clarity and is non-uniform in appearance.

As above stated, for the subsequent treatment caustic potash solution of about 30° Baumé at room temperature may be employed, or caustic soda solution may be used in concentrations of 6 to less than 12° Baumé with subsequent rapid removal of the caustic to correct this lack of clarity and non-uniformity. The control of the process is more easily effected by the use of caustic potash.

The following examples are illustrative of the process. It is to be understood that these examples are illustrative and the invention is not restricted thereto except as indicated in the appended claims.

*Examples*

1. Viscose muslin which has been pre-cleaned by the usual methods and dried under tension is passed in the broad state through sulfuric acid of 48° Baumé (measured at 15° C.). The temperature of the acid is kept between -1° C. and +1° C.; the time of action amounts to 11 seconds. Immediately thereafter the acid is washed out with water at room temperature, and any possible residues of acid are neutralized besides with dilute ammonia. The fabric is now freed from the excess of water by pressing or suction, and in still moist condition is then exposed for 6 seconds to the action of caustic potash solution of 30° Baumé, freed from caustic by means of hot water at about 70° C., acidified with sulfuric acid of 1° Baumé, and washed. The material can now be either blued or dyed by the usual methods, whereupon it is dried under tension in the directions of warp and weft; expediently it is further stentered before the drying.

In this way one obtains an extensively translucent, comparatively but little stiffened fabric. The clarity and uniformity of the fabric picture are considerably improved in comparison with a material that has only been parchmentized with acid.

2. Viscose muslin that has been imprinted with dyes fast to acid and fast to alkali is exposed for 12 seconds to the action of sulfuric acid cooled to +5° C., whose specific gravity measured at 15° C. amounts to 47° Baumé, is then washed neutral and dried under tension. Now the material is immersed for 10 seconds at 15 to 20° C. in caustic potash solution of 25° Baumé, freed from caustic with hot water (about 70° C.), acidified, and washed until a neutral reaction is attained. After pressing-off of the excess water, the material is dried under tension. The drying of the material can be effected on a tension frame.

After the above treatment sequence, one obtains a variegated fabric with greatly increased transparency; in the imprinted parts a deepening of color takes place.

3. A fabric produced from spun rayon of high wet tenacity, for example, No. 80 Eng., is desized, soaped, bleached, dyed, and dried on a tension frame.

Now one passes it through a parchmentizing bath of the following composition:

|                                       | Per cent |
|---------------------------------------|----------|
| Sulfuric acid calculated as $H_2SO_4$ | 59.6     |
| Urea                                  | 14.8     |
| Water                                 | 25.6     |

The temperature of the bath is kept at 25° C.;

the time of action amounts to 16 seconds. Immediately thereafter the material is washed cold, and the moist material is then subjected to after-treatment with caustic potash solution of 28° Baumé for 8 seconds at room temperature. After the freeing from caustic and washing with hot water, the material is stentered and dried under tension. Advantageously, the material is finally calendered besides.

10. Spun rayon muslin that has been treated in this manner corresponds in appearance to a high-grade cotton organdy.

15. Viscose spun rayon muslin is, in accordance with the usual methods, singed, desized, boiled, bleached, dried on a tension frame, and imprinted with a resist of the following composition:

|                  | Grams |
|------------------|-------|
| Titanium dioxide | 260   |
| Acetyl cellulose | 40    |
| 20. Acetone      | 500   |
| Phenol           | 150   |
| Water            | 50    |
|                  | 1000  |

25. Now the material is exposed in the open width for 10 seconds to the action of sulfuric acid of 47° Baumé. In this process the temperature of the acid should be kept at 10° C. After the complete washing-out of the acid, the material is subjected to after-treatment with caustic potash solution of 30° Baumé for 6 seconds at room temperature, washed hot, neutralized, and dried under tension.

30. In this way one obtains highly contrasting patterns of white opaque printed areas on a transparent ground.

35. Viscose voile is parchmentized at 10° C. for 15 seconds with phosphoric acid of 55° Baumé (measured at 15° C.), and immediately thereafter is subjected to after-treatment with caustic potash solution as described in Example 4 and dried under tension.

40. There results an extensively transparentized, moderately stiffened fabric.

45. 6. Viscose marquisette is pre-cleaned by the well-known methods and dried on a tension frame. Now the material is passed in the open width through 60% sulfuric acid to which per liter 10 cc. of 40% technical concentrated formaldehyde have been added. The temperature of the acid should be 0° C., the time of action 12 seconds. After the washing out of the acid, the material is dried under tension, whereupon it is subjected to after-treatment with caustic soda solution of 8° Baumé for 5 seconds, is washed hot, acidified, and thoroughly rinsed. Finally the fabric is tensed in the warp and weft directions and dried.

50. An extensively transparent fabric is obtained.

55. 7. A light weight fabric consisting in warp and weft of cuprammonium silk yarns is pre-cleaned by the well-known methods and dried on a tension frame. Now the material is treated in the open width for 12 seconds with sulfuric acid of 47.5° Baumé at a temperature of 0° C. After washing out the acid the fabric is exposed for 6 seconds to the action of caustic potash solution of 28° Baumé, washed with hot water to remove the caustic, acidulated with sulfuric acid of 1° Baumé, washed until a neutral reaction is attained, stentered and dried under tension.

60. There results a highly transparent, moderately stiffened fabric.

70. 8. Spun rayon muslin containing effect yarns

or twists of cotton is singed, desized, boiled, bleached and dried on a tension frame. Now it is treated with sulfuric acid of 47° Baumé as described in Example 4, and after complete washing out of the acid, exposed to the action of caustic soda solution of 10° Baumé for 8 seconds, washed with hot water, acidified and washed until a neutral reaction is attained. Finally the fabric is stentered and dried under tension.

There results a transparent fabric containing nontransparentized effect yarns giving interesting optical contrasts.

The fabrics obtained in accordance with the above examples have a uniform appearance where an all-over effect is obtained and the same uniformity may be observed in the transparent patterned goods. In addition the goods are of high quality, are relatively soft, and of marketable character.

The expression "regenerated cellulose material" as employed in the claims refers to regenerated cellulose in the form of fiber, yarns, and fabrics of such material.

What I claim is:

1. A process which comprises treating regenerated cellulose with an aqueous solution selected from the group consisting of sulfuric acid of about 42° to about 48° Bé., phosphoric acid of about 50° to about 55° Bé., hydrochloric acid of the order of 20° Bé., zinc chloride of the order of 50° Bé. and calcium thiocyanate of the order of 25° Bé. for a period of time of the order of 10 seconds at a temperature in a range of about room temperature and below, whereby an acid parchmentized regenerated cellulose textile material results which lacks clarity and is non-uniform in appearance, and treating such material substantially free from acid at room temperature with an aqueous caustic alkali solution selected from the group consisting of potassium hydroxide of the order of 30° Bé. and sodium hydroxide at 6° to less than 12° Bé. for a period of the order of 10 seconds to produce a clear uniform transparent fabric.

2. A process which comprises treating regenerated cellulose with an aqueous solution of sulfuric acid of about 42° to about 48° Bé. for a period of time of the order of 10 seconds at a temperature in a range of about room temperature and below, whereby an acid parchmentized regenerated cellulose textile material results which

lacks clarity and is non-uniform in appearance, and treating such material substantially free from acid at room temperature with an aqueous caustic alkali solution selected from the group consisting of potassium hydroxide of the order of 30° Bé. and sodium hydroxide at 6° to less than 12° Bé. for a period of the order of 10 seconds to produce a clear uniform transparent fabric.

10 3. A process which comprises treating regenerated cellulose with an aqueous solution of phosphoric acid of about 50° to about 55° Bé. for a period of time of the order of 15 seconds at a temperature in a range of about room temperature and below, whereby an acid parchmentized regenerated cellulose textile material results which lacks clarity and is non-uniform in appearance, and treating such material substantially free from acid at room temperature with an aqueous solution of potassium hydroxide of about 30° Bé. for a period of the order of 6 seconds to produce a clear uniform transparent fabric.

20 4. A clear, uniform, transparent fabric of regenerated cellulose produced by the process of claim 1.

ERNST WEISS.

#### REFERENCES CITED

30 The following references are of record in the file of this patent:

#### UNITED STATES PATENTS

| Number       | Name          | Date           |
|--------------|---------------|----------------|
| 35 1,558,453 | Barrett       | Oct. 27, 1925  |
| 1,812,204    | Hall          | June 30, 1931  |
| 1,985,124    | Weiss         | Dec. 18, 1934  |
| 1,989,100    | Lilienfeld    | Jan. 29, 1935  |
| 1,989,101    | Lilienfeld    | Jan. 29, 1935  |
| 40 1,998,577 | Heberlein     | Apr. 23, 1935  |
| 2,085,946    | Bodmer et al. | July 6, 1937   |
| 2,174,534    | Shipp         | Oct. 3, 1939   |
| 2,200,792    | Hefti         | May 14, 1940   |
| 2,202,200    | Haller et al. | May 28, 1940   |
| 45 2,215,938 | Schonholzer   | Sept. 24, 1940 |
| 2,245,123    | Belloc        | June 10, 1941  |

#### FOREIGN PATENTS

| Number     | Country       | Date          |
|------------|---------------|---------------|
| 50 464,965 | Great Britain | Apr. 28, 1937 |
| 516,843    | Great Britain | Jan. 12, 1940 |